

## UNITED STATES PATENT OFFICE

VICTOR R. ABRAMS, OF BRUNSWICK, GEORGIA, ASSIGNOR OF ONE-HALF TO ADOLPH N. SHELANDER, OF BRUNSWICK, GEORGIA

## PROCESS FOR WOOD PRESERVATION

No Drawing.

Application filed November 19, 1927. Serial No. 234,566.

The present invention relates to the preservation of wood, and has particular reference to treating wood in the form of piling, timbers, railroad ties, planks and the like, which are to come into contact with sea water, for preventing the destruction caused by marine insects such as *Teredo*, *Limnoria* and the like.

I desire to call attention to the fact that wood, for piling and for other uses in which it is permanently or temporarily in contact with sea water, is subject to attacks by various forms of animal life, such as the *Teredo* and *Limnoria*, barnacles and various others, which bore into the wood, thereby weakening the wood, and greatly shortening the life of the wood under these conditions. Also in some locations, animals such as termites eat into wood which is not in contact with sea water, such as railroad ties, sills of buildings or houses, door steps and the like, this being particularly noticeable in the case of wood which is close to the ground or on the ground, and which is accordingly more or less damp. In some localities, particularly in the south, railroad ties are frequently injured in this manner.

In accordance with the present invention, I preferably treat the wood first with a solution of copper sulphate, by impregnation, after which the excess of copper sulphate solution which has not been absorbed is removed from the wood, or from the treating vessel, and then the wood is impregnated with a solution of a soluble resinate, whereby an insoluble copper resinate is formed. In some cases more than two successive treatments with these two substances alternately may be employed, and it will be understood that the copper salt or the resinate can be applied first as desired, and the invention is not restricted to any particular order of treatment with these two materials.

When the wood is in a green or wet condition, it may first be steamed and subjected to a vacuum, in order to dry the wood and to open the pores thereof. When the wood is dry, it may first be subjected to a vacuum in order to drive out the air from the pores of the wood, as much as possible.

Assuming the wood to be in an air tight cylinder or vessel under vacuum, for the purpose of withdrawing the air from the pores of the wood, in which operation a vacuum of say 18 to 25 inches more or less, may be employed, depending upon the conditions, and the wood may be hot or cold as desired, there is then introduced into the said receptacle, a solution of a rosin soap. This solution may be a 5% solution of sodium resinate, although stronger or weaker solutions can be used if desired. The solution is run in preferably sufficiently to completely submerge the wood, after which fluid pressure is applied, say by pumping in more of the sodium resinate solution, in order to cause the wood to become permeated with the sodium resinate solution. When sufficient impregnation has been produced, the pumping will be stopped and the unabsorbed liquid is pumped out of the treating receptacle into a storage tank. Steaming and, or, a vacuum is preferably applied at this stage, in order to draw out more or less of the resinate solution, which is likewise pumped into the storage tanks.

An aqueous solution of a soluble copper salt, such as copper sulphate, say 2 to 10% strength, is then pumped in, and pressure is then applied upon the solution to force the copper sulphate solution into the wood, preferably sufficiently to thoroughly permeate the wood. The copper sulphate reacts with the sodium resinate in the wood, to produce insoluble copper resinate, and after sufficient impregnation with the copper sulphate solution, the excess is drawn off, and the wood may then be considered as completely treated, and may be dried either by steam and vacuum, or by merely stacking up the wood in the atmosphere or under a shed. Generally I recommend continuing the operation, by giving a second treatment with the rosin soap solution, similarly to the above, in order to neutralize the remaining copper sulphate, and to increase the amount of copper resinate in the pores and cavities of the wood. The treatments may be continued as many times as desired, alternating between the rosin soap and the copper sulphate solution or other solution of a soluble copper salt, but for ordi-

55  
60  
65  
70  
75  
80  
85  
90  
95  
100

nary purposes two, three or four treatments, will be found to give a sufficient impregnation.

As a modification of the invention, I may 5 employ in the first step, say a solution of a resinate, then a solution of copper sulphate, and then a solution of ordinary soap (for example a soap made from caustic soda and tallow or other form of grease). Instead of 10 using resinate solution alone, I may employ mixtures of rosin with various oils and greases for producing the initial soap.

I have above referred to the use of copper salts such as copper sulphate. It is how- 15 ever within the scope of the invention, to employ salts of other metals having toxic properties or insect destroying properties, such as arsenic, tin, zinc, mercury and the like.

It will be further understood that in some 20 instances it may be advisable to employ a solution of a soluble resinate, then say a copper salt, then a soluble carbonate or hydroxide, which react with the excess of copper, producing a mixed precipitant in situ of 25 the wood.

The process presents certain advantages 30 over the prior processes of using creosote oil, heavy petroleum oil and the like, in that the preservation seems to be more perma- 35 nent, and the materials used are much cheaper than creosote and similar substances. Wood impregnated with creosote is also objectionable as having a disagreeable odor, and also because the active constituents of the 35 creosote seem to be sufficiently soluble to be leached out of the wood, in water, after a time.

I call attention to the fact that the impreg- 40 nation may be carried to any depth as desired, and in ordinary practice, it is possible to car- 45 ry the impregnating solution clear to the heart of the timber. In ordinary practice there will be much more of the copper resinate, etc., precipitated in the outer por- 50 tions of the wood, than in the inner portions, which is really an advantage because the in- 55 sects and other organisms have to enter the wood from the exterior. When planking, boards and other sawed timber is to be em- 50 ployed, it is preferably treated after sawing, in order to produce the said effect.

I call attention to the fact that the toxic 55 properties of the copper compounds also pre- 60 vent the action of fungi, spores and bac- 65 teria which produce decay.

The invention also contemplates the alter- 60 nate impregnation of the wood with solutions of soluble soaps and with soluble salts of the heavy metals other than sodium, potassium, lithium, calcium, and ammonium.

Also I may employ solutions of ordinary 65 soaps, such as the oleates, stearates, linoleates, rhionoleates, tungoleates and other fatty oils entirely to replace the resinate solu- 65 tions in the manner described above.

I claim:—

1. A process of preserving wood in the form of piling, timbers, railroad ties, planks, and the like, which comprises the step of forming copper resinate in situ in the pores 70 of the wood.

2. A process of preserving wood in the form of piling, timbers, railroad ties, planks, and the like, which comprises the step of forming copper resinate throughout sub- 75 stantially the entire body of the wood, the deposit of copper resinate being more concentrated in the outer parts of the pieces of wood.

3. In the preservation of wood in the form 80 of structural articles the steps of alternately impregnating the wood with a soluble copper salt and a soluble resinate separately introduced into the pores of the wood, whereby an insoluble copper resinate is formed in situ 85 in the cavities of the wood.

4. A process of preserving wood by the alternate impregnation with solution of soluble soaps and with an aqueous solution of soluble copper compounds separately intro- 90 duced into the pores of the wood.

5. A process of preserving wood by the alternate impregnation with solutions of soluble soaps and with an aqueous solution of soluble salts of the heavy metals, the solu- 95 tions being separately introduced into the pores of the wood.

In testimony whereof I affix my signature.

VICTOR R. ABRAMS.

100

105

110

115

120

125

130